

# UNITED STATES PATENT OFFICE.

GIACOMO BOSIO AND ANTONIO PERADOTTO, OF TURIN, ITALY.

## METHOD OF TANNING HIDES.

1,266,203.

Specification of Letters Patent. Patented May 14, 1918.

No Drawing.

Application filed April 19, 1916. Serial No. 92,272.

To all whom it may concern:

Be it known that we, GIACOMO BOSIO and ANTONIO PERADOTTO, both subjects of the King of Italy, residing at Turin, in Italy, have invented a certain new and useful Improved Method of Tanning Hides, of which the following is a specification.

This invention relates to an improved method of tanning hides by means of tannin 10 or tannic solutions.

In the method hitherto employed of tanning hides by means of tannin or solutions containing tannin, the hides after washing, cleansing, etc., are immersed in a succession 15 of vats containing more or less weak tannic solutions.

This method requires considerable labor and time—the gradations of the tannic liquors of the first baths being always very 20 low about  $\frac{1}{2}$  degree and those of the last baths reach 4 to 5 per cent. Constant manipulation of the skins is also required in each vat. The hides remain 15 to 20 days in each vat and on removal are submitted 25 to additional tanning in tan-pits or by means of rotating drums or other apparatus requiring the expenditure of mechanical or hand power, and containing more or less strong baths, thus necessitating considerable 30 time for these different treatments.

The present invention relates to an accelerated tanning method (based on the employment of tannin or tannic solutions) allowing of obtaining perfectly tanned hides 35 in a time varying from one day for thin hides to 15 days for the heaviest hides according to the quality of the hides and their thickness while using for this effect vats only.

40 The general idea which guided the inventors is that the skin intended to be transformed into leather has been during the life of the animal at an even temperature varying with the nature of the class of animal, for instance approximately 36° C. Consequently it is at the life temperature that the tanning operation should be effected in order that the tanning action is produced while the skin retains all the elasticity of 45 the fiber and the natural quantity and density of the gelatin, that is to say, when it is in the best condition.

The method also consists in submitting the skins to be treated to very strong gradations of tannin at this relatively high tem-

perature, the gelatino-tannic combination being produced under conditions which most approach the skin in the vital state and producing a compact and homogeneous leather.

Acting on this principle, the skins (after the washing and cleansing process which must be very carefully effected) are placed in a vat containing concentrated tannic solution heated to the said life temperature 60 of the respective animals, say, for instance, 34 to 36°; it must be stated however that the skins must not be plunged immediately into baths of this temperature but the bath must be brought progressively though 65 quickly to the said temperature after the skins are immersed in order to prevent the sudden great difference of heat between the operations of cleansing and tanning which might harm the skins under treatment. The 70 bath should be heated up to the desired temperature in a relatively very short time, say not more than  $\frac{1}{2}$  of an hour.

As in the known methods the skins could be suspended in the vats on battens or frames 80 fixed or movable, and these vats may either be separate or if desired placed in progressive communication in order to otherwise insure a relative movement and constant friction of the liquid against the skins, the 85 important points being that the skins immersed in the solutions must remain well stretched and without creases, while however there is constant relative movement with respect to the tannic solution.

In the improved method the skins are thus 90 immersed in tannic solution of a strong gradation and heated to the life temperature and maintained at that temperature during practically the whole of the process.

This gradation of the liquid can vary (according to the product to be obtained) from 95 6 to 25° Baumé corresponding to 7 to 35% of extract of tannin without addition of other pseudo-tanning matter and without 100 alteration of any kind according to the quality of the skins to be treated. These, (suspended on frames or battens kept in movement so that they may be kept stretched and free from creases are thus capable of 105 being kept in relative movement as regards the liquid or are capable of withstanding the movement of the liquid relative to them), are immersed in the cold tannic liquid above indicated, liquid and skins then being 110

brought to the life temperature of the animal which is thereafter maintained during the treatment.

The baths are prepared by means of dry extract, using any suitable apparatus for such preparation, this extract comprising 60 to 70% of tannin. Liquid extracts of high concentration could also be used.

The skins should remain in the vats without being removed therefrom during the tanning operation. This operation will vary between 1 to 15 days according to the thickness and the quality of the skins; after this time the hides obtained are ready to receive any kind of finishing work.

*Examples.*

1. To tan leather intended for sole leather it is necessary to employ during the process 20 a kilogram of extract containing 30 to 31% of tannin for each kilogram of hide after the skins have been washed, stripped of hair and flesh, cleaned and finally drained. This quantity of extract is necessary to fix 25 all the gelatin contained in the fibers of the skin when a firm compact and impermeable leather is to be obtained.

2. For leathers intended for harness making, saddlery, etc., or intended to be employed in a more or less soft condition such as for uppers for shoes and boots as the leathers are then charged with greasy substances, the quantity of tannin employed during the process varies between 600 and 35 900 grams per kilogram of hide in the dressed condition as in the previous example, according to the thickness of the leathers and the finish they are to have.

The advantages of the improved method 10 are essentially the following:—

1. *Economy of time.*—The time employed being at the maximum 15 days for very heavy hides is insignificant with regard to that necessitated by the old system which 45 might comprise entire years.

2. *Manipulation.*—This is *nil* during the operation; the skins do not require to be manipulated during the whole time that the tannin treatment lasts.

3. *Economy of motive power.*—The use of the fuller being suppressed the manipulation of which necessitates constant work, there is only the heating of the bath to be effected, which can be obtained very economically without manipulation solely by the exhaust from steam heaters.

4. *Output.*—By the favorable conditions obtained by the combination of the heat and of the gelatino-tannic reactions by the use of 60 concentrated tannic liquor, an output of 60 to 62% calculated on the weight of the skins is obtained instead of 50% obtained with the old tanning method.

5. *Quality of product.*—Finally the hides 65 obtained by this process of tanning have

not their fibers deteriorated, their elasticity remains perfect and their strength is much greater as the following comparative dynamo-metrical tests made on hides treated by the known processes and by the present 70 process show. The resistances to rupture per square sectional millimeter are—

|                                                                |           |    |
|----------------------------------------------------------------|-----------|----|
| For leathers for machine belting<br>treated by the old process | 3 kg. 300 | 75 |
| For the same leathers treated by<br>the present process        | 3 kg. 400 |    |
| For sole leathers treated by the<br>old processes              | 2 kg. 300 |    |
| For similar leathers treated by<br>the present process         | 2 kg. 600 | 80 |

If it is desired to give the leathers treated by the present method the appearance obtained by the old tanning methods they can after being tanned in the manner stated, be 85 submitted to complementary operations which do not come within the scope of the present invention.

What we claim as our invention and desire to secure by Letters Patent of the 90 United States is:—

1. The method of tanning hides consisting in treating them in stationary vats containing tannic solutions, without addition of any other acting agent than tannin, at a 95 concentration of 7 to 35% of extract of tannin according to the quality and thickness of the skins to be treated, the skins being immersed in the cold tannic solution the temperature of the bath together with 100 the skins immersed therein being thereupon raised in a relatively short time to that of the animal during its life and maintained practically at said life temperature, without removing the skins until the completion of 105 the tanning.

2. The method of tanning hides consisting in treating them in stationary vats containing tannic solutions, without addition of any other acting agent than tannin, at a concentration corresponding from 7 to 35% of extract of tannin according to the quality and thickness of the skins to be treated, the skins being secured on battens or frames and immersed in the cold solution of tannin, 115 the temperature of the bath together with the immersed skins being raised gradually or progressively, in a relatively short time to that of the animal, whose skin is treated, during its life, and maintained at said life 120 temperature for a period varying from 1 to 15 days, without removing the skins from the vats, means being provided for relative movement of the battens or frames and of the bath.

3. The method of tanning hides consisting in treating them in stationary vats containing tannic solutions, without addition of any other acting agent than the tannin, at a concentration corresponding from 7 to 130

35% of extract of tannin according to the quality and thickness of the skins to be treated, the tannic solution being constantly kept in movement and the skins being secured on fixed battens or frames and also being immersed in the cold tannic solution kept in movement, and the temperature raised gradually and quickly, that is to say progressively and in a relatively short time, 10 to the temperature of the live body heat of the animal whose skin is being treated and maintained practically at said live body

temperature and without removing the skins from the vats for a period varying from 1 to 15 days, substantially as set forth. 15

In witness whereof we have signed this specification in the presence of two witnesses.

GIACOMO BOSIO.  
ANTONIO PERADOTTO.

Witnesses:

NORAH WHITESTONE,  
TRANCHINO AUG.